

## UNITED STATES PATENT OFFICE

CLYDE C. DE WITT, OF HOUGHTON, MICHIGAN

## MOLDING MATERIAL

No Drawing.

Application filed April 8, 1929. Serial No. 353,696.

- This invention relates to materials such as are employed for making molds in which molten metal is to be cast, the principal object being the provision of a synthetic molding material that will be efficient and satisfactory in use, and economical to produce. Another object is to provide a synthetic molding material comprising a mixture of sand and iron ore.
- 10 Another object is to provide a molding material comprising a mixture of gel-coated sand and iron ore, the latter of which may also be provided with a gel-coating.

15 A further object is to provide a molding or core material comprising a mixture of sand and iron ore which has been treated with a solution of iron hydrosol to provide the individual grains or particles thereof with a coating of iron hydrogel.

20 The material now universally used in making molds for the casting of molten metal is a sand-clay mixture known as molding sand which is found in the natural state in various parts of the country. These natural molding sands are found in beds of varying thicknesses, and the clay, together with other material which forms the binder for the sand, varies in proportion from the top to the bottom of the bed. Consequently some portions 25 of the bed may be too rich in binder, while other portions may be lean in binder. This condition as to the whole bed may sometimes be remedied by thoroughly mixing all portions of the strata, but even in such cases the final product may not be of the best quality desired and very often such mixture is not complete so that various parts of the mass may have different characteristics than other parts. Furthermore, in view of the fact that 30 the extent of such beds of natural molding sand is relatively limited throughout the country, this sand is relatively expensive and the freight charges necessary to bring it from its point of deposit to the foundry often run 35 into a relatively large figure. Accordingly, I have provided a synthetic molding material which may be employed in the place of natural molding sands for substantially all molding operations. This material is such 40 as to be capable of being produced at a rela-

tively small cost at any point where a supply of relatively clean sand is available.

In molding operations where cores are employed, it is necessary in accordance with present day molding practice to treat the sand with suitable so-called core oils, and bake the formed cores in order to provide them with the requisite rigidity. Furthermore, these baked cores are not susceptible to the influence of water and consequently are relatively difficult to remove from castings having relatively complicated core work in them. The material provided by the present invention may be employed for cores without the addition of the so-called core oils or the subsequent baking operation, and may be readily and easily removed from the castings by simply flushing them out with water.

25 The material I employ in the present case is a mixture of sand and iron ore. The sand may be of a relatively varied nature. It may comprise sand of the natural molding type that is deficient in natural binders, or it may be substantially naked sand, such as shore sand or any other sand that is suitably cleaned so as to remove any earth or any other foreign matter that may be mixed therewith in the natural state. The iron ore that I prefer to employ may be either hematite, or limonite, such as is found in inexhaustible quantities in the natural state in various parts of the country. The size of the particles of iron ore may vary according to the permeability desired in the final product, the greater the permeability the larger the particles of iron ore employed, as will be readily understood to those skilled in the art.

30 The sand and iron ore, either separately or mixed with each other, are subjected to a solution of iron hydrosol so that each particle is provided with a coating of iron hydrogel. The thickness of the coat may be controlled by the number of applications of iron hydrosol. If a relatively thick coat is desired the 35 particles may be dried or partially dried and then subjected again to the action of the iron hydrosol and this may be repeated until the desired thickness of coat is acquired. If the sand and iron ore are coated separately 40

from each other, they must of course be thoroughly intermixed after coating.

5 The particles of iron ore and sand may be treated with the iron hydrosol in any desired manner, that is, the particles may be settled through the solution, or the solution may be allowed to filter through the particles, or an amount of the solution may be added to a mass of the particles and the particles mixed or milled to obtain the proper distribution.

10 Once used, these particles of iron hydrogel-coated sand and iron and hydrogel-coated iron ore may be gathered up again, partially dried, formed into appropriate molds and used for the same purpose many 15 times without further treatment with iron hydrosol. When revivified by the hydrosol treatment the coated sand and coated iron ore particles need not be separated.

20 The strength of any such mixture, moist or dry, depends upon the contacting area between the particles. The function of the hydrogel in the moist state is to provide means of intimately contacting adjacent particles.

25 In the moist state the strength is due mainly to the tensile strength of water at the contact points to the grain packing and to the percentage of moisture. When the material is packed in the moist condition the hydrogel 30 films coalesce. As these coalesced films dry their particles become both interlocked and cemented. The particles which have been separated in a dry state must of course be moistened and time must be allowed for the 35 gelatinous coatings to swell so that the coalescence of the films will be accomplished again when the material is packed.

This material may be employed as a core sand without the addition of any core oils 40 and without a baking process. Used as a core sand this material is quite hard when packed moist and air-dried, and is sufficiently refractory for a number of foundry operations. After the metal is cast around the core the 45 removal of the core is accomplished by simply wetting the core material with water. The mixture of the sand and iron ore may then be shaken out of the casting or more easily flushed out with a stream of water. In fact, 50 if an air-dried or even a baked core of this material is thrust into a glass of water it will literally fly apart, due either to the eagerness of its component materials to absorb water or to the capillary forces brought into play by 55 presenting small orifices to the water, through which the water rises into the capillaries and in doing so wets the particles forming the capillary walls to such an extent that the mass disintegrates into its original small particles. 60 This characteristic of this material effects a considerable saving in foundry practice.

The material herein specified will perhaps be found more satisfactory for use in connection with metals having a relatively low melting point for the reason that if it is heated

on too high a temperature the mixture of iron oxide and silica tends to react to form iron silicate. For metals having a relatively low casting temperature this objection has little, if any, application.

70 It is to be noted that any refractory material having a grain size similar to that of sand may be used as described above in place of the sand, and it is not my intention to limit the present application solely to the use of sand and iron ore, and in the following claims where the term "sand" is employed, it is to be understood as meaning not only sand as it is ordinarily known, but any refractory or like grain size that may be employed in its stead. 75

It may also be noted that other metallic hydrosols may be employed in place of the iron hydrosol to impart a gelatinous coating to the grains of sand and iron ore and I, therefore, do not limit myself specifically to the use 80 of iron hydrosol.

Where iron hydrosol is to be employed I prefer that it be employed as a relatively cold solution having a pH value of from 4.5 to 6.2 pH. The iron hydrosol solution may 90 be prepared in the following manner. Allow a dilute solution of ferric chloride to dissolve all the hydrated iron oxide or ferric hydroxide that it can when the temperature of the solution is approximately 90° to 100° C. 95 When properly prepared, such a solution will contain approximately one part of ferric chloride to fifteen parts iron oxide. The resultant colloidal solution will be a clear, amber-colored liquid. The pH value of the iron hydrosol may be adjusted by means of suitable neutralizing agents or buffers, the function of which can be obtained from any text-book on physical or electro-chemistry. 100

Other methods of preparing iron hydrosol 105 may be used equally well, but inasmuch as the present invention does not relate to the preparation of the same, it is not thought necessary to describe the same here.

Formal changes may be made in the specific embodiment of the invention described without departing from the spirit and substance of the broad invention, the scope of which is commensurate with the appended 110 claims.

115 What I claim is:

1. A material for making molds for metallic castings comprising a mixture of sand and iron ore.

2. A material for making molds for metallic castings comprising a mixture of sand and iron ore, said sand having an artificial coating of gel insoluble in water.

3. A material for making molds for metallic castings comprising a mixture of sand and iron ore, said sand having an artificial coating with an artificial gel coating.

4. A material for making molds for metallic castings the bulk of which comprises a mixture of sand and iron ore the individual 120

particles of which are provided with an artificial gel coating substantially insoluble in water.

5. A molding material comprising a mixture of sand and iron ore the particles of which are provided with an artificial coating of iron hydrogel.

10. An article of manufacture comprising a synthetic molding material composed of a mixture of sand and iron ore, the individual particles of the iron ore being provided with an artificial coating of iron hydrogel.

15. An article of manufacture comprising a synthetic molding material composed of naturally substantially naked sand grains and iron ore the particles of said sand being provided with an artificial coating of iron hydrogel.

20. An article of manufacture comprising a synthetic molding material composed of shore sand and iron ore which have been treated with iron hydrosol.

25. In the manufacture of an artificial molding material composed of particles of sand and iron ore, the step of subjecting said particles to the action of an iron hydrosol solution having a pH value of from 4.5 to 6.2.

CLYDE C. DE WITT.

30

#### CERTIFICATE OF CORRECTION.

Patent No. 1,770,688.

Granted July 15, 1930, to

CLYDE C. DE WITT.

It is hereby certified that error appears in the printed specification of the above numbered patent requiring correction as follows: Page 2, line 126, claim 3, strike out the words "said sand having an artificial coat" and insert instead the particles of which are provided; and that the said Letters Patent should be read with this correction therein that the same may conform to the record of the case in the Patent Office.

Signed and sealed this 24th day of February, A. D. 1931.

(Seal)

M. J. Moore,  
Acting Commissioner of Patents.

particles of which are provided with an artificial gel coating substantially insoluble in water.

5. A molding material comprising a mixture of sand and iron ore the particles of which are provided with an artificial coating of iron hydrogel.

10. An article of manufacture comprising a synthetic molding material composed of a mixture of sand and iron ore, the individual particles of the iron ore being provided with an artificial coating of iron hydrogel.

15. An article of manufacture comprising a synthetic molding material composed of naturally substantially naked sand grains and iron ore the particles of said sand being provided with an artificial coating of iron hydrogel.

20. An article of manufacture comprising a synthetic molding material composed of shore sand and iron ore which have been treated with iron hydrosol.

25. In the manufacture of an artificial molding material composed of particles of sand and iron ore, the step of subjecting said particles to the action of an iron hydrosol solution having a pH value of from 4.5 to 6.2.

CLYDE C. DE WITT.

30

### CERTIFICATE OF CORRECTION.

Patent No. 1,770,688.

Granted July 15, 1930, to

CLYDE C. DE WITT.

It is hereby certified that error appears in the printed specification of the above numbered patent requiring correction as follows: Page 2, line 126, claim 3, strike out the words "said sand having an artificial coat" and insert instead the particles of which are provided; and that the said Letters Patent should be read with this correction therein that the same may conform to the record of the case in the Patent Office.

Signed and sealed this 24th day of February, A. D. 1931.

(Seal)

M. J. Moore,  
Acting Commissioner of Patents.